

J. SANDERS.

MANUFACTURING SOUND RECORD TABLETS.

APPLICATION FILED FEB. 6, 1909.

1,179,660.

Patented Apr. 18, 1916.



Witnesses

  
F. G. Chapman.

Inventor

  
Joseph Sanders.

By

  
C. Brown & Co.

Attorneys

UNITED STATES PATENT OFFICE.

JOSEPH SANDERS, OF WASHINGTON, DISTRICT OF COLUMBIA.

## MANUFACTURING SOUND-RECORD TABLETS.

1,179,660.

Specification of Letters Patent. Patented Apr. 18, 1916.

Application filed February 6, 1909. Serial No. 476,419.

To all whom it may concern:

Be it known that I, JOSEPH SANDERS, a citizen of the United States, residing at 770 Girard street, in the city of Washington and District of Columbia, have invented a new and useful Improvement in Manufacturing Sound-Record Tablets, of which the following is a specification.

10 This invention has reference to improvements in the manufacture of sound record tablets and more particularly in the manufacture of sound record tablets of the type disclosed in my application No. 204,024, filed April 20, 1904, for improvements in sound record tablets.

15 sound record tablets.  
In the type of tablet disclosed in the said application there is provided a basic disk of cardboard, or strawboard, or pulpboard, or other such fibrous material and this basic disk  
20 is sized with a material capable of softening under heat and then yielding to pressure, but which is quite hard and resistant when cold, that is at normal temperatures, and which furthermore cements the fibers of the  
25 disk together so that, when the base has been coated with a suitable record material and a sound record matrix is pressed against the same while both the coating and the disk are heated so that the coating and  
30 sizing have become appropriately softened and the basic disk has become more or less condensed by the pressure used, the sizing will hold the compressed base in the condensed condition after the sizing has become  
35 hardened by the chilling of the tablet before the pressure is relieved.

The present invention relates more particularly to the manufacture of the basic disks upon which the coating of record material is either directly applied as in the aforesaid application or is first applied to a thin carrier such as a sheet of paper and then the coated sheet is applied to the fibrous, sized base as set forth in my application No. 239,961, filed January 6, 1905, for gramophone record tablets.

In accordance with the present invention, disks of the proper size, agreeable to the sizes of commercial forms of sound record tablets, are first cut or punched from pulp-board, or strawboard, or cardboard, or any other of the materials suitable for the purpose but which for convenience of description will be considered as included in the generic term cardboard. Of course the disks may be molded into shape from suitable

stock and thus the waste due to cutting or  
punching from sheets of the material is  
avoided. Since the cardboard disks are  
liable to or do actually contain some mois-  
ture they are now dried in order to expel  
any moisture which they may contain. The  
disks are now ready for treatment with a  
suitable sizing which sizing should, for the  
purposes of the invention, be sufficiently ad-  
herent to the fibers making up the card-  
board disk to cement these fibers together  
even against considerable force tending to  
separate the fibers. Furthermore the sizing  
should be characterized by being compara-  
tively hard and resistant at ordinary tem-  
perature so as not to yield under the han-  
dling to which record tablets are ordinarily  
subjected, but which will soften, under a  
degree of heat low enough not to injure the  
material entering into the composition of  
the record receiving surface, to a sufficient  
degree to yield under the pressure to which  
the tablet is subjected in the operation of  
pressing a record groove into the record re-  
ceiving surface from a matrix of the sound  
record.

record. There are various compositions suitable for the sizing, such for instance as those named in the aforesaid applications for Letters Patent, but I have found Manila gum to be a most excellent substance for the purpose, and since the gum is applied in accordance with the present invention when dissolved in a suitable solvent, I have obtained very satisfactory results when the gum is dissolved in wood alcohol and benzol in the proportion of eighty pounds of Manila gum to forty-six pints of wood alcohol and fifty pints of benzol, it being understood however, that these proportions may be varied without disadvantage. Since the materials used as bought in the open market are not always free from dirt, it is advisable to filter the solution. 85 90 95 100

In order to apply the solution of sizing to the disks they are placed in a vacuum chamber, preferably in baskets suitably shaped to support the disks on edge and present practically the entire exterior of the disks to the action of the sizing solution. The air is extracted from the chamber in which the disks are placed, this chamber of course being capable of being sealed against the entrance of air and as the air is extracted from the chamber such air as may be imprisoned within the disks is also extracted. The sizing so-

lution is now allowed to flow into the vacuum chamber to a depth sufficient to immerse completely the cardboard disks within said chamber and under these conditions the sizing penetrates the innermost interstices of the disks thus thoroughly infiltrating them, even to the intercellular structure. The vacuum chamber is now opened and the impregnated disks are removed, the baskets or supports for the disks having maintained them separated one from the other so that the infiltration was thorough and expeditious. The infiltrated disks are now stacked with or without separators but preferably without separators, and are placed in a press and subjected to pressure, say from thirty-five to forty tons total for disks which are about ten inches in diameter. This causes the surplus sizing to be squeezed out and such surplus sizing may be caught in a suitable receptacle and returned to the reservoir of the sizing solution or may be allowed to flow spontaneously to the reservoir through a suitable conduit. Of course the expressing of the surplus sizing solution may be accomplished either by a press as the term is ordinarily understood or the disks may be passed through pressing rolls which may be properly spaced and adjusted for the same purpose.

When the pressure is relieved each disk will return toward its normal thickness, having been reduced in thickness by the applied pressure. This will cause the re-absorption of any of the sizing which remains on the surface or edges of the disks and does not flow away therefrom so that the surface becomes relatively dry and thus permits easy handling of the sized disks even though a large portion of the solvent is still retained in the disks and the sizing is still in a sticky or tacky condition.

By regulating the pressure to the fluidity of the sizing solution or by suiting the amount of solvent employed to the pressure used, the amount of sizing in the disks after the surplus has been removed may be fixed to a nicety. The amount of sizing used should be such that after the final compression of the tablet under the pressure used for impressing the sound record groove into the tablet from a matrix thereof there will be neither material surplus nor lack of sizing in the basic disks. The proportions of the ingredients of the sizing solution and the pressures employed as hereinbefore given are those used in actual practice and are very close to if not actually the exact proportions of ingredients for the sizing solution, and very close to the pressures needed for the best results with pulpboard disks.

After the disks have been infiltrated with the sizing solution and the surplus removed in the manner described the disks are dried.

Since air drying would be very slow the disks are dried in an oven or in a vacuum chamber and if so desired the solvent used in the sizing solution may be recovered in the usual manner.

The dried disks with the sizing therein are liable to be more or less distorted from a true flat shape and sometimes these disks contain hard spots incorporated in the material from which the disks are cut or punched, during the manufacture of such material. In order to flatten out the disks, and also to flatten the hard spots, the disks are again heated to a sufficient degree to soften the sizing and are then subjected to a moderate pressure, say from five to ten tons total for a ten inch disk. For this step separators may or may not be used. Separators are not always necessary even when hard spots are present or suspected, but may be used, if needed, to flatten out hard spots in some kinds of cardboard. The separators, when used either in the step just named or when the disks are first subjected to pressure, may be metal disks of suitable diameter and suitable thickness, sheet metal being thick enough for the purpose. The disks having been cooled under the pressure used in the last described step remain flat and of even thickness indefinitely. The disks may now, if desirable or necessary, have the edges rounded off or smoothed in a lathe and are ready to receive the surface coating of any desired suitable record receiving material in any suitable manner. The methods set forth in my aforesaid application for Letters Patent No. 204,024, or in the aforesaid application No. 239,961, or in my application No. 410,456, filed January 11, 1908, for sound record tablets and method of manufacturing the same, with the materials specified in said several applications, will give most excellent results.

As a specific instance of a surfacing material adapted for the reception and reproduction of a sound record of the gramophone type, there may be prepared a mixture of shellac and natural oxid of iron in about the proportions set forth in my Letters Patent No. 787,001, granted April 11, 1905, for a composition of matter for sound record tablets. The shellac may be incorporated with the powdered oxid of iron on hot mixing rolls and after cooling the material may be powdered. Then by coating the disk with a thin solution of shellac or with what may be termed an emulsion of the material just described made by dissolving the shellac in a solvent, while the oxid of iron remains in suspension in the solution, the powdered record material may be deposited in a thin layer on the still wet coating which then acts to cement the powdered material to the basic disk. This method of applying the record receiving material to the basic disk

and also the specific material mentioned is to be taken as illustrative only since various other materials and other methods of applying the materials to the basic disk may be employed. It may be stated however, that the particular material mentioned and the method of application thereof gives very satisfactory results.

The method of producing a sound record 10 groove from a matrix of an original sound record in a tablet having a surface coating of record receiving material on a basic disk sized with a material which softens under heat consists in heating such tablet until the 15 surface coating and the sizing have become sufficiently softened and then applying pressure with the matrix against the face of the tablet thus impressing the matrix into the softened facing layer. The fibrous portion of the base or under-structure being 20 incompletely filled with the sizing, will condense under the action of the pressure until the interstices of the fibrous base are substantially filled with the sizing, or at least 25 so filled that when the tablet has cooled to the normal atmospheric temperature, which is usually accomplished by chilling the mold in which the matrix and tablet are placed for compression, the fibers making up the 30 fibrous base are all cemented together by the sizing.

The finished tablet with the sound record groove impressed is indistinguishable in appearance from a record tablet made wholly 35 from record material, but the tablet with the fibrous base or under-structure is materially lighter than the solid record tablet and far more resistant to breakage. Moreover, the base or understructure or core of the 40 finished tablet has substantially the same coefficients of bending and expansion as the surface coating of gramophone record material, wherefore cracking of the surface material and warping of the tablets is avoided. 45 The base or core is also resonant, so that there is no deadening of the sound in reproduction thereof from the complete sound record tablet. The operation of pressing the matrix into the record surface and the 50 resultant tablet is not materially different from the method of procedure and the result obtained when the record receiving material is first applied to a paper carrier and the paper carrier so coated is then applied 55 to the basic sized disk.

In the accompanying drawing forming a part of this specification there is shown a diagram in which the various steps already described are briefly set forth in order, and 60 since these steps have all been hereinbefore fully set forth the description need not be repeated with special reference to the schematic representation of the drawing.

Instead, however, of applying the sizing 65 in solution to the base, or in addition to the

use of a solvent, the sizing may be brought to a flowing condition by heat. The fibrous disks are then immersed in the hot sizing and are afterward pressed while the sizing is still hot enough to flow, or after reheating 70 if desired, to expel the surplus sizing and to cause the reabsorption of adherent sizing, after which the disks are cooled either spontaneously or by being chilled. When the disks are sized by a sizing brought to a flowing condition by heat, they are not dried 75 after the reabsorption of the adherent sizing, but are merely cooled, and distortions due to the evaporation or expelling of a solvent are avoided.

What is claimed is:

1. The method of producing basic disks or understructures for sound records, consisting in infiltrating a fibrous base with a solution of a normally hard sizing and subjecting the infiltrated base to such heavy pressure as to discharge surplus sizing solution and on relief of the pressure cause such reabsorption of the solution as to render the surface of the base dry enough for 90 handling.

2. The method of producing basic disks or understructures for sound records, consisting in infiltrating a fibrous base with a solution of a thermoplastic sizing and subjecting the infiltrated base to such heavy pressure as to discharge surplus sizing solution and on relief of the pressure cause such reabsorption of the solution still on the surface of the fibrous base as to render said 100 surface dry enough for handling.

3. The method of producing basis disks or understructures for sound record tablets, consisting in subjecting a fibrous base to subatmospheric pressure and infiltrating it with a solution of a thermoplastic sizing and then subjecting the infiltrated base to such heavy pressure as to discharge surplus sizing solution and on the relief of the pressure cause the reabsorption of sizing solution on the surface of the infiltrated fibrous base to an extent to thereby render the surface of the base dry enough for handling.

4. The method of producing basic disks or understructures for sound record tablets, consisting in infiltrating a fibrous disk with a solution of normally hard sizing capable of softening under heat and before the solvent has evaporated subjecting the disk to heavy pressure simultaneously applied to substantially the whole area of the disk and then relieving the pressure and thereby causing reabsorption of sizing solution still on the surface of the disk to an extent to render the surface of the disk dry 120 enough for handling.

5. The method of producing basic disks or understructures for sound record tablets consisting in infiltrating a fibrous disk with a solution of a resinous sizing in a 130

volatile solvent, then subjecting the infiltrated disk to heavy pressure simultaneously applied over substantially the whole area of the disk to discharge surplus sizing solution, then relieving the pressure to thereby cause reabsorption of sizing solution still on the surface of the disk to an extent to render the surface dry enough for handling and then subjecting the disk to 10 heat to evaporate the solvent.

6. The method of producing basic disks or understructures for sound record tablets, which consists in extracting the air from the immediate neighborhood of a base, 15 then infiltrating the base with a sizing in solution, then subjecting the infiltrated base to heavy pressure to force out a portion of the absorbed sizing solution, and then relieving the pressure and thereby causing 20 the base to re-absorb substantially all the sizing solution then on the surface thereof.

7. The method of producing basic disks or understructures for sound record tablets, which consists in extracting the air from 25 the immediate neighborhood of a base, then infiltrating the base with a thermoplastic sizing in solution, then subjecting the infiltrated base to heavy pressure to force out a portion of the absorbed sizing solution, 30 and then relieving the pressure and thereby causing the base to re-absorb substantially all of the sizing solution then on the surface thereof.

8. The method of producing basic disks or understructures for sound record tablets, which consists in first drying a base, 35 then extracting the air from the immediate neighborhood of the base, then infiltrating the base with a thermoplastic sizing in solution, then subjecting the infiltrated base to heavy pressure to force out a portion of the absorbed sizing in solution, and then relieving the pressure and thereby causing 40 the base to re-absorb any sizing solution on the surface thereof to render such surface dry enough to handle.

9. The method of producing basic disks or understructures for sound record tablets, which consist in extracting the air from 50 the immediate neighborhood of a base, then infiltrating the base with a thermoplastic sizing in solution, then subjecting the infiltrated base to heavy pressure to force out a portion of the absorbed sizing solution, 55 then relieving the pressure and thereby causing the base to re-absorb the sizing solution on the surface thereof to an extent to render the surface dry enough to handle, and then causing the evaporation of the solvent and the consequent solidification of the sizing.

10. The method of producing basic disks or understructures for sound record tablets, which consists in infiltrating a fibrous 65 disk with thermoplastic sizing, then soft-

tening the sizing by heat, and then straightening or flattening the disk by pressure while the sizing is plastic and maintaining the pressure until the sizing has solidified by cooling.

11. The method of producing basic disks or understructures for sound record tablets, which consists in infiltrating a fibrous disk with thermoplastic sizing, then softening the sizing by heat, and then straightening or flattening the disk by pressure against surfaces unyielding to the pressure used while the sizing is plastic, and maintaining the pressure until the sizing has solidified by cooling.

12. The method of producing basic disks or understructures for sound record tablets, which consists in infiltrating a fibrous base with a solution of a thermoplastic sizing in a vacuum chamber, then subjecting the infiltrated base to pressure to force out a portion of the absorbed sizing solution, then relieving the base from pressure to cause the re-absorption of sizing clinging to the surface of the base, then causing the removal of the sizing solvent from the base, then heating the base to soften the sizing, and then subjecting the heated base with the softened sizing to pressure.

13. The method of producing tablets for the reception of sound record impressions from matrices of the same, which consists in infiltrating a fibrous base with thermoplastic sizing, then softening the sizing by heat, then straightening or flattening the base while the sizing is plastic by pressure applied to said base and maintaining the pressure until the sizing has solidified by cooling, and then applying a surface coating of suitable sound record material.

14. The method of producing tablets for the reception of sound record grooves from a matrix of the same under the action of heat and pressure, which consists in infiltrating a fibrous disk with thermoplastic sizing, then softening the sizing by heat, then straightening out or flattening the disk by pressure applied while the sizing is plastic and with the disk against surfaces unyielding to the pressure used, and maintaining the pressure until the sizing has solidified by cooling, and then applying a thermoplastic sound record material to the surface of the tablet.

15. The method of producing sound record tablets which consists in infiltrating a fibrous disk with thermoplastic sizing, then softening the sizing by heat, then while the sizing is plastic pressing the disk against surfaces unyielding to the pressure used and maintaining the pressure until the sizing has solidified by cooling, then coating the sized disk with thermoplastic record material, and finally impressing a sound record groove into the record material from a ma-

trix of a sound record while the tablet is softened by heat.

16. The method of producing sound record tablets which consists in first producing 5 disks of fibrous material, then infiltrating the disks with a solution of a thermoplastic sizing, then subjecting the infiltrated disks to pressure to force out a portion of the sizing solution, then relieving the pressure, and permitting the disks to swell to 10 re-absorb sizing solution clinging to the surface of the disks, then causing the solidification of the sizing in the disk by the evaporation of the solvent thereof, then 15 heating the sized disks, then flattening the disks by pressure while the sizing is softened by heat, then coating the disk with a suitable record material, and finally producing 20 a sound record groove in the record receiving surface from a matrix of such sound record under the action of heat and pressure.

17. A step in the method of preparing sound record tablets, which consists in subjecting 25 fibrous basic disks containing thermoplastic sizing to the action of heat and pressure before the application of the record receiving surface.

18. A step in the method of preparing sound record tablets, which consists in subjecting 30 fibrous basic disks containing thermoplastic sizing to the action of heat and pressure against surfaces resistant to the action of the heat and pressure used and before 35 the application of the record receiving surface.

19. The method of producing basic disks or understructures for sound record tablets, which consists in infiltrating a fibrous base 40 with a sizing, and while the sizing is in a condition to flow expressing surplus sizing, then relieving the pressure to cause reabsorption of sizing clinging to the surface of the base, and then causing the solidification 45 of the sizing and subjecting the solidified base to pressure.

20. The method of producing basic disks or understructures for sound record tablets, which consists in infiltrating a fibrous base 50 with a sizing in solution and while the sizing is in a condition to flow, expressing surplus sizing, then relieving the pressure to cause reabsorption of sizing clinging to the surface of the base, then heating the sized base to drive off the solvent and then subjecting the base to pressure.

21. The method of producing basic disks or understructures for sound record tablets, which consists in impregnating such disk 60 with a sizing, then expressing surplus sizing, then relieving pressure, then subjecting the sized base to the action of a vacuum and heat, and then while the sized base is hot subjecting the base to pressure.

65 22. The method of producing basic disks

or understructures for sound record tablets, which consists in infiltrating a fibrous base with sizing, then while the sizing is in a condition to flow, expressing surplus sizing, then relieving the pressure to cause reabsorption of sizing clinging to the surface of the base, then subjecting the sized base to the action of sub-atmospheric pressure and heat, then while the base is hot, subjecting it to pressure, then coating the base with thermoplastic sound record material and then producing thereupon a sound record from a matrix of the same under the action of heat and pressure.

70 23. The method of producing basic disks or understructures for sound record tablets, consisting in infiltrating the disks or understructures with a solution of resinous sizing, placing a plurality of the sized disks or understructures in face to face relation, 75 pressing the disks or understructures together to express surplus sizing, and then relieving the pressure to cause reabsorption of any sizing still on the surfaces, all while the sizing is still in solution.

80 24. The method of producing basic disks or understructures preparatory to coating them with gramophone record material, consisting in infiltrating the fibrous bases with a solution of a sizing which is hard 85 and resonant when cold and plastic when heated and also has expansion and bending coefficients substantially like those of gramophone record material, grounding the infiltrated bases face to face, applying pressure to the ends of the group to compress the bases and thereby express sizing solution therefrom, and then relieving the pressure and permitting the bases to return toward the uncompressed condition to 90 cause reabsorption of any sizing clinging to the surfaces of the bases.

95 25. The method of preparing basic disks or understructures for sound record tablets, which consists in infiltrating fibrous bases 100 with a solution of resinous sizing, and then rendering the surfaces of the bases relatively dry by stacking the infiltrated bases and compressing the stack to express surplus sizing and then relieving the pressure 105 to permit the bases to return toward the uncompressed condition and thereby reabsorb any expressed sizing solution still on the surfaces of the bases.

110 26. The method of producing sound record tablets which consists in first producing cardboard disks, then infiltrating the disks with thermoplastic sizing in solution, then subjecting the infiltrated disks to pressure to discharge surplus sizing solution, then relieving the pressure to cause reabsorption of sizing solution on the surface of the disks, then evaporating the solvent to cause solidification of the sizing in the disks, then 115 coating the disks with suitable record ma- 120

terial, and finally producing a sound record groove in the record material from a suitable matrix under the action of heat and pressure.

5 27. The method of producing sound record tablets, which consists in infiltrating a cardboard base with thermoplastic sizing and while the sizing is in a condition to flow expressing surplus sizing and causing 10 reabsorption of any sizing on the surface of the base to render such surface free enough from sizing for handling at once, coating the base with sound record material and producing thereupon a sound record 15 from a matrix of the same under the action of heat and pressure.

28. The method of producing sound record tablets, which consists in producing disks of cardboard, infiltrating them under 20 subatmospheric pressure with a solution of

resinous sizing, stacking the infiltrated disks and subjecting them to heavy pressure to discharge surplus sizing solution, relieving the pressure to cause reabsorption of any sizing clinging to the surfaces of the 25 disks to an extent to render them sufficiently surface-dry to permit handling, heating the disks to evaporate the solvent of the sizing, coating the disks with record receiving material and impressing a sound record matrix into the record material under the action of heat and pressure. 30

In testimony that I claim the foregoing as my own, I have hereto affixed my signature in the presence of two witnesses.

JOSEPH SANDERS.

Witnesses:

F. T. CHAPMAN,  
E. DANIELS.